

Dec. 5, 1933.

A. E. PEW, JR

1,937,782

LUBRICATING OIL

Filed Jan. 13, 1928

3 Sheets-Sheet 1



WITNESS:

Robert R. Kitchell

INVENTOR

Arthur E. Pew, Jr.

BY

Busser and Harding

ATTORNEYS.

Dec. 5, 1933.

A. E. PEW, JR  
LUBRICATING OIL

1,937,782

Filed Jan. 13, 1928

3 Sheets-Sheet 2



FIG. 3.



FIG. 2.

WITNESS:

Bob P. Kitchel.

INVENTOR

Arthur E. Pew, Jr.  
BY  
Buser and Harding  
ATTORNEYS.

Dec. 5, 1933.

A. E. PEW, JR

1,937,782

LUBRICATING OIL

Filed Jan. 13, 1928

3 Sheets-Sheet 3



FIG. 4.



FIG. 5.

WITNESS:

John P. Mitchell.

Arthur E. Pew, Jr.

BY  
Bauer and Harding  
ATTORNEYS.

## UNITED STATES PATENT OFFICE

1,937,782

## LUBRICATING OIL

Arthur E. Pew, Jr., Bryn Mawr, Pa., assignor to  
 Sun Oil Company, Philadelphia, Pa., a corpora-  
 tion of New Jersey

Application January 13, 1928. Serial No. 246,446

13 Claims. (Cl. 196—151)

The object of this invention is the production, as distillates, of very high boiling point lubricating oils of fairly wide cuts having a combination of qualities, particularly low carbon content, good 5 color, low organic acidity and good demulsibility, that has never heretofore characterized any distillates from petroleum.

The manufacture of low and medium boiling point lubricating oil distillates with flash and fire 10 points characteristic of such oils and having low carbon content, good color, low organic acidity tests, good demulsibility tests in accordance with the Herschel method, and substantially free of cracked products, presents, in the present advanced state of the art, no serious problems.

It is also possible to produce fairly high boiling point distillates having the desired qualities specified in greater or less degree. It is also possible to produce such distillates as narrow cuts, but 20 the production of narrow cuts on a commercial scale is not economically practicable.

Some of the factors that are necessary or helpful to the production of high boiling point distillates are well understood. Thus, it is well known that by the use of steam, the boiling points of 25 the oil fractions may be substantially reduced, thereby substantially reducing the formation of cracked products—cracking being a factor of time and temperature; but even moderately high boiling point oils produced by distillation with steam at atmospheric pressure or a low vacuum are objectionable because of the resultant discoloration of the oil. This discoloration is largely the result 30 of the production of cracked products, the reduction in boiling point not being sufficient to avoid substantial cracking. It is also in part attributable to the formation of products of oxidation, which not only discolor, but unfavorably affect other qualities of, the oil.

So far, however, as concerns oxidation products, it is well understood that the introduction 40 into the oil of an acid neutralizer, such as caustic soda or other alkali, tends to prevent their formation, or to neutralize them, and thereby more or less materially reduce discoloration.

It is also well understood that by the use of an extremely high vacuum, the boiling point of the oil may be very much reduced, whereby all but the highest boiling point fractions may be 50 distilled off at so low a temperature that cracking will be minimized or substantially prevented.

It is also known that, as the pressure on the oil, in distillation, approaches an absolute vacuum, the boiling point of the oil falls at a continually 55 accelerating rate. That is, if the fall of the boil-

ing point, with reduction in absolute pressure, be graphically represented by a line intersecting vertical and horizontal lines indicating respectively progressively lower absolute pressures and progressively lower boiling points, the line will be 60 a curve something like that shown in Figs. 4 and 5 of the drawings. This knowledge has been available to the art, and the consequent advantage of distillation under an extremely high vacuum has been known, since the publication of the work of 65 Weilandt and Kraft, Berichte, etc., vol. 29, page 1323 (1896), and vol. 38, page 263 (1904).

Those skilled in the art, since the date of these publications, and possibly earlier, have been well aware of this accelerating drop in boiling point as 70 an absolute vacuum is approached, and patentees, in describing processes of distilling oil under vacuum, have expressed the desirability of employing as high a vacuum as possible. Until within the past eight or ten years, however, engineering 75 difficulties have prevented the maintenance of an extremely high vacuum in the oil circulating system.

There are other factors, however, that have prevented the operativeness of very high vacuum 80 processes in the production of very high boiling point distillates with very high flash and fire tests and substantially devoid of cracked products. Thus, it has not been appreciated that the absolute pressure to which the oil of an oil body 85 is subjected depends not alone, or even mainly, upon the absolute pressure in the superincumbent vapor space but depends also upon the depth of the body of oil. Thus, if the existence of a body of oil of approximately .8 sp. gr. at 500° F. 90 and two feet in depth, under an absolute vacuum, be assumed, the hydrostatic pressure on the oil at the bottom of the column will be about 33 mm. mercury absolute. Assuming the boiling point of the oil on the surface of the body to be about 95 500 degrees F., the boiling point of the oil at the bottom of the column will be about 600 degrees F. Consequently, the boiling point of a substantial part of the oil body will be greatly above what the boiling point of the oil would be if the factor 100 of hydrostatic pressure could be eliminated.

Principally for this reason, although very high vacuum processes, as applied to batch processes, have gone into commercial use and have produced high boiling point distillates of good quality, they 105 have not successfully produced the very high boiling point distillates that the art demands and which it is the object of this invention to produce.

However, distilling apparatus in which the oil was widely distributed over a heated surface 110

(with resultant elimination of the factor of hydrostatic pressure) while the oil was subjected to a vacuum was disclosed as early as the date (December 10, 1867) of the Twedde Patent No. 72,125; but no practical use has ever been made of such an apparatus to effect the distillation of high boiling point distillates of the desired characteristics and qualities. Indeed, it is questionable whether the process can be successfully practiced in such an apparatus; there being other factors that must coexist with an extremely high vacuum and the dispersal of the liquid oil over the heating surface, in order to successfully produce such boiling point distillates. The principal of these other factors is probably the selection of a heating agent having a high rate of heat transfer in order to maintain the smallest practicable temperature difference between the oil and the heating medium. Ordinary heating media, such as furnace gases and condensable or superheated steam, having a comparatively low rate of heat transfer, must have a temperature so far exceeding the desired boiling point of the oil to be distilled that local overheating of the oil occurs, resulting in cracking and the consequent production of a distillate having so high a content of products of decomposition as to render the whole process unworkable to produce high boiling point distillates of the desired characteristics and qualities. It has been found that the use of mercury vapor as a heating medium, provided it transfers its latent heat of condensation, meets the requirements if other necessary factors are present. Thereby a temperature difference between the oil to be distilled and the temperature of condensation of the mercury vapor may be maintained well under 50° F., thus avoiding local overheating. For mercury vapor it may be possible, in some cases, to substitute another vaporizable metal, or perhaps a vaporizable metallic compound or alloy, or some other substance, such as diphenyl oxide, benzophenone, or sulfur.

Still other conditions must or should coexist with those named in order to successfully produce the high boiling distillates hereinafter described.

Heat should be applied only to the liquid oil and not to the vapors. If no heat is applied to the vapors, they tend to cool immediately after leaving the surface of the oil body. If, on the other hand, they are directly heated by the heating medium, conditions most favorable to cracking, if cracking is possible at the temperature to which the vapors are subjected, are produced; it having been demonstrated that oil in a vapor state is more readily cracked than oil in a liquid state, some authorities holding that the cracking of oil can proceed only when the oil is in a vapor state.

Slightly prolonged contact between the liquid oil being heated and the oil vapors should be avoided, this also being a condition productive of cracking of the oil vapors.

The oil vapors, when condensed, produce a distillate containing fixed gases that produce an objectionable odor. The distillate should be subjected to a deodorizing process in order to remove these fixed gases.

The oil to be distilled must not be subjected to any preliminary processes, such as the driving off of benzine, gasoline, kerosene, gas oil, fuel oil, or lower boiling lubricating distillates, that crack the oil, since the high boiling oils whose production is the object of the invention cannot be produced even though a substantial cracking temperature is avoided in their distillation, if the oil contains

cracked products to begin with. All such preliminary operations should be conducted, as far as possible, under non-cracking and non-oxidizing conditions. If, however, the crude oil contains cracked products, or a limited amount of cracked products are produced in preliminary operations, the use of an acid neutralizing agent, such as caustic soda, is necessary, even where all the other conditions required for successful operation are present.

Unless all, or most, of the conditions hereinbefore recited coexist in the process, the production of the oils forming the subject-matter of this invention is impossible. It is, therefore, important that the conditions required to produce them should be recapitulated, as follows:

1. The subjection of the oil, while it is being vaporized, to a very high vacuum, which should preferably be equivalent to a pressure of from one to seven millimeters mercury absolute, although this absolute pressure may be exceeded in the production of high boiling point oils within the lower parts of the ranges of the boiling points, flash tests and fire tests hereinafter specified.

2. The subjection of the oil to the vaporizing operation for the shortest practicable time.

3. The avoidance of a column of oil of any substantial height, thereby making the factor of hydrostatic pressure negligible.

4. The use of a heating agent that will make possible a small temperature difference between it and the oil, say not exceeding, and preferably substantially less than, about 50° F., so as to avoid local overheating.

5. The application of heat, principally, if not wholly, to the liquid oil, and the avoidance of conditions whereby the vapors, when formed, are subjected to the temperature conditions required to form them.

6. The avoidance of prolonged contact between the liquid oil being heated and the vapors that have escaped from the liquid oil body.

7. Treatment of the crude oil in such manner as to insure the absence, or elimination, of cracked or oxidized products from the stock from which the very high boiling point oils are to be distilled.

8. The deodorization of the distillate.

It will be understood that all these conditions advantageously may, but need not, coexist in the production of oils having average boiling points, and flash and fire tests, below those embodying the present invention; and that such oils, having substantially the other desirable qualities and characteristics hereinbefore enumerated, may be produced by other processes. The present invention is confined to lubricating oil distillates having qualities and characteristics heretofore unknown in distillates, and combinations of qualities and characteristics heretofore unknown in any oil, whether a residue or a distillate, and which have been produced by a process, also heretofore unknown, having all the features hereinbefore enumerated; and while it is not asserted that no such novel distillates can be produced by any process varying therefrom, a knowledge of such process, and of an apparatus for carrying out the process, is necessary to enable those skilled in the art to produce the new distillate. For this reason, a brief description of such process and apparatus is advisable, and drawings, in which such apparatus is set forth in sufficient detail, are herewith appended.

Fig. 1 is a diagram, in sectional elevation, of a part of a distilling plant in which the improved

distillates may be produced, showing particularly the means for heating the lubricating stock.

Fig. 2 is a diagram, in sectional elevation, of that part of the plant in which lubricating stock is distilled and the distillate refined.

Fig. 3 is a longitudinal section through one of the stills of Fig. 2.

Figs. 4 and 5 are diagrams illustrating the fall of the boiling point with reduction in absolute pressure.

A complete apparatus, including means for preparing the lubricating stock from crude oil in order to prepare a lubricating stock free of cracked or oxidized products, and for distilling off lubricating fractions, is set forth in an application filed by me January 8, 1927, Serial No. 159,754. The present apparatus constitutes a part of the apparatus therein disclosed.

It may be assumed that the oil which is to be subjected to the treatment required to produce the high boiling distillates which form the subject of the present invention is a high boiling residue of Texas asphalt base crude, which has been deprived of all its (relatively) lower boiling constituents, including all the low boiling and medium boiling lubricating fractions and, indeed, including also what the art recognizes as high boiling lubricating fractions. What is left is composed, either wholly or in large part, of a residue that has never before been distilled without such substantial cracking as to make the distillate unfit for use as a lubricating oil unless reduced with steam and fire, and subsequently treated, at a comparatively high cost, and which resultant lubricating oil is inferior in fire and flash tests and lacks also the combination of other qualities which it is the object of this invention to produce. It should, also, be understood that these oil fractions from which inferior distillates have been heretofore produced at high cost comprise the most valuable lubricating constituents of the crude, and which, when isolated as a distillate, command prices much higher than that of any other heretofore known lubricating oil distillate.

From a mercury boiler *a* extends a mercury vapor line *b* having branches extending to the mercury chambers *d* of two vaporizers 9 and 10. In the production of new oils, the use of two vaporizers, in which successively higher boiling point fractions are evaporated, is advisable, in that a satisfactory commercial product can be made from a mixture of the two distillates. Each branch pipe is equipped with a valve *c*, by means of which the flow of mercury vapor into the mercury vapor chamber *d* of either vaporizer, 9 or 10, may be independently regulated. Extending from the mercury chamber *d* of each vaporizer is a mercury condensate return *e*. From the mercury vapor supply line *b* extends a pipe *f* communicating with a pressure control valve *g*, which opens when the boiler pressure exceeds a predetermined maximum and allows mercury vapor to flow past the valve into a condenser *h*, which communicates, through a pipe *h'*, with the boiler *a* either direct or through the mercury condensate return *e*.

Each vaporizer, 9 or 10, comprises a long tubular container divided, by means of a pan or partition *i* running lengthwise therethrough, into the specified mercury vapor condensing chamber *d* and an oil vaporizing chamber *j*. The oil flows onto and down over and along pan *i* in a comparatively thin stream and at a fairly rapid rate. A fraction of the oil is vaporized in each vaporizer. If a sufficiently high boiling stock is run

into vaporizer 9 and if the temperatures are properly regulated, the fraction vaporized in vaporizer 10 is of so high a boiling point that the residue constitutes practically nothing but asphalt, which may be sold as such, or further refined to improve its quality. There need be no waste intermediate product.

For the two vaporizers may be substituted, as above stated, a single long vaporizer, and if two or more distillates of progressively higher boiling points are desired, progressively higher boiling point vapors may be taken off at different points along the length of the vaporizer, and fractionally condensed. It is preferred to use two vaporizers in order to provide a minimum effective temperature difference between the oil in each vaporizer and the mercury vapor in each vaporizer. It is also permissible to use more than two vaporizers. In any case, however, it is desirable to provide a number of vapor exit pipes *k* along the length of each vaporizer so as to allow the vapors to freely and quickly escape as soon as they leave the surface of the liquid oil body.

Connected with the oil vaporizing chamber of each vaporizer is a condensing, refluxing and deodorizing apparatus, which will now be described.

The vapor from pipes *k* flows into a header *m* and thence through pipe *n* to the lower part of a tower *o*. Above the discharge mouth of pipe *n* is a grid *p*, which supports chemical tiles, such as Raschig rings, *r*. Above and spaced from tiles *r* is another grid *s*, which supports another pile of tiles *t*.

Below grid *s* and above tiles *r* is provided a deflector *u* and an orificed pan *v* through which oil vapors can flow upwardly and which is adapted to receive reflux condensate, which is carried off through pipe 20.

The bottom of the tower communicates, through pipe *w*, with the oil feed end of one of the vaporizers, 9 or 10, preferably the same vaporizer as that from which the oil vapors pass into the bottom of the tower.

The top of the tower communicates, through a pipe *x*, with a stink oil receiver *y*, to which is connected a pipe *z* connected with vacuum.

Any vapors carried into tower *o* that are heavier than the fraction which it is desired to segregate will condense while going through tiles *r* and flow down to the bottom of the tower. Any particles of oil that may be entrained with the vapors will also flow to the bottom of the tower.

The uncondensed vapors will flow up through pan *v*, grid *s* and tiles *t*, wherein the vapors are cooled and most of them condensed. Uncondensable gases escape through pipe *x* into receiver *y*. The condensate flows back through tiles *t* and grid *s* into receiver *v*, whence it flows through pipe 20 into a deodorizer 21.

Deodorizer 21 comprises a chamber provided with staggered flow plates 22 over which the distillate is thinly distributed and down which it flows at a speed sufficient to create a substantial turbulence. Outlet pipes 23 connect with a header 24, which connects with vacuum. The bottom of chamber 21 connects, through a pipe 26, with a receiver 27, which connects, through a pipe 28, with vacuum.

In the deodorizer, odoriferous gases are removed from the oil on each plate 22 and are withdrawn through pipes 23; the arrangement being such that there can be no reabsorption of gases in the oil.

The oil passing into receiver 27 is ready for the market without further treatment.

The vapors leaving the vaporizer 9 or 10 are thus subjected to partial reflux condensation and to deodorization, by removal of odor producing gases, first, in the tower o and finally in the deodorizer 21.

The final residue from the oil vaporizer chamber j of vaporizer 10 flows into a tank 30, which may be connected to vacuum through pipe 31.

The highest degree of vacuum, which may be equal to an absolute pressure of (say) one to five millimeters mercury, is that operative on the deodorizer 21, and receivers 30, y and 27, particularly on the deodorizer. Without objectionably large connecting pipes, there is some drop in vacuum between the vacuum pumps and the oil vaporizing chambers of the vaporizers, particularly if a refluxing and condensing tower is used. It is quite possible, however, to maintain a pressure in the oil vaporizers of from two to ten millimeters mercury absolute. If a very wide range of cut is desired, the tower o may be eliminated and a fractional condenser substituted and the heavier condensate passed to the deodorizer, thence to storage. It is possible to maintain, in the vaporizers, if desired, a degree of vacuum more nearly equal to that at the vacuum pumps than where a tower o is employed.

The importance of maintaining in the vaporizers a degree of vacuum as near as possible to an absolute vacuum may be appreciated by reference to the charts, Figs. 4 and 5. In each figure, the vertical lines indicate absolute pressures mm. mercury, the line at the extreme right indicating atmospheric pressure and the horizontal lines indicate the boiling points. The curves are those worked out for oils whose boiling points are respectively 500° C., 400° C., and 300° C. In Fig. 5 the absolute pressures are indicated logarithmically in order to more clearly show the differences in boiling points in the very low pressure range. Fig. 4 shows more clearly the accelerated rate at which the boiling point falls as an absolute vacuum is approached.

From this diagram it will be clear that in the operation of the described apparatus, if it is desired to produce the very highest boiling distillates, a reduction in absolute pressure to substantially below ten mm. mercury is quite necessary, and a reduction, if possible, to, or even below, one or two mm. mercury is desirable.

In producing distillates embodying this invention, it is essential that the lubricating stock fed to vaporizer 9 should be stock that has been divested of its lower and medium boiling lubricating fractions. Preferably, such lubricating fractions are removed by passage through a series of vaporizers (which may be, for example, eight in number) like vaporizers 9 and 10, wherein, however, the establishment of a very high vacuum is not essential, because, even in the last vaporizer of the series preceding vaporizers 9 and 10, the temperature to which the oil is raised does not exceed the temperature at which, with the absolute pressure maintained therein, substantial cracking begins. It should also be understood that I do not necessarily contemplate the production of the new oil in vaporizer 9. The new oil is preferably the product of vaporizer 10, or is a blend of the products of vaporizers 9 and 10.

As an example of one way of producing the new oils, let it be assumed that an asphalt base oil, such as Texas crude, has been subjected to a succession of distillation processes under such conditions as prevent the substantial production of cracked products, and that the oil has been de-

prived of all its lighter constituents and of the major part of its lubricating fractions, leaving a residue containing, in addition to asphalt, only the higher boiling fractions which it is desired to separate as distillates. Thus, it may be assumed that, before the introduction of residual oil to vaporizer 9, the distillation process has involved the subjection of the oil, in the immediately preceding vaporizer, to a temperature of 609-650° F. at some pressure between atmospheric and one inch mercury absolute, that all or most of the fractions that distil off at that temperature and pressure have been distilled off, and that the residual oil is free of coke and other cracked residues. Or it may be assumed that the residual oil contains high boiling fractions which, if isolated as a composite distillate, will have, as an example, a gravity of 17.8, a flash point of 510-515° F., a fire point of 595-600° F., and a viscosity of 149/210°. In other words, all that it is necessary to assume is that the residual oil entering vaporizer 9 contains high boiling fractions all or a large part of which are those which it is the object of this invention to separate out as distillates.

Such a residual oil is now run through vaporizers 9 and 10, under the conditions prescribed: namely, the use of a heating agent which, like mercury vapor, is capable of transferring its latent heat of condensation at a temperature not greatly exceeding the boiling point, at a very high vacuum, of the highest boiling fraction that is to be vaporized; the maintenance on the oil being vaporized of a very high vacuum equivalent to an absolute pressure of (say) two to ten millimeters mercury, and preferably as low as possible, especially in vaporizer 10; the avoidance of hydrostatic pressure; the subjection of the oil to the heating agent for only the limited time required for the oil to traverse the length of the pan; the direct transfer of heat (through the pan) only to the liquid oil; and the free escape of the vapor; all as hereinbefore described.

The distillate obtained from vaporizer 9 may or may not be an oil embodying this invention; that is, it may or may not have all the characteristics, hereinafter described, of the new oil. Thus, it may have a flash point of 470° F. or somewhat less, a fire point of 550° F. or somewhat less, and a viscosity of 120 at 210° F.; or the flash and fire points and viscosity may be much higher. The distillate obtained from vaporizer 10, however, does have all these characteristics in such maximum degree that, when blended with the distillate from vaporizer 9 in (say) about equal proportions, it produces an oil which has such novel characteristics in a less pronounced degree and which is more readily marketable than the distillate from vaporizer 10.

Bearing in mind that the oil in vaporizer 10 is distilled so as to leave a residue comprised mainly or wholly of asphalt, the following are examples of different distillates obtained from vaporizer 10.

|          | Gravity | Flash   | Fire    | Viscosity | 140 |
|----------|---------|---------|---------|-----------|-----|
| I-----   | 18.4    | 535° F. | 625° F. | 177/210°  |     |
| II-----  | 17.7    | 540° F. | 640° F. | 196/210°  |     |
| III----- | 17.4    | 555° F. | 625° F. | 226/210°  |     |
| IV-----  | 17.8    | 575° F. | 660° F. | 254/210°  |     |

It should be stated that the viscosity characteristics of the distillate are subject to wide variation and depend primarily on the kind of crude which is run through the plant.

It should also be understood that such characteristics as the gravity, and the flash and fire points, of a distillate from the final vaporizer depend on the proportion of the highest boiling fractions that have been abstracted from the oil before it enters the final vaporizer. Thus, by increasing the number of vaporizers, so as to decrease the amount of the highest boiling oil that is vaporized in the last vaporizer, the distillate therefrom may be made to have flash and fire tests even higher than those characterizing distillate IV; and the same result may be accomplished by careful fractional condensation of the

any distillates heretofore produced from mineral oil. They are, indeed, so much higher than is required for any ordinary purposes that they can advantageously be blended with a lower boiling distillate, such as, for example, the distillate from vaporizer 9. The following is a distillation analysis of a blend of the latter distillate with the three distillates I, II and III from vaporizer 10:

Gravity 17.8; flash 510°; fire 600°; viscosity 149/210.

Charge 1200 cc. No soda.

Initial 460—566 at 2 mm.

| 15 | Cut | Temp. |      | Pres. | Am't.   | Chg. | Crude grav. | Flash | Fire | Viscosity | C.T.  | Color N.P.A. | 90  |
|----|-----|-------|------|-------|---------|------|-------------|-------|------|-----------|-------|--------------|-----|
|    |     | Vap.  | Liq. |       |         |      |             |       |      |           |       |              |     |
| 20 | 1   | 526   | 568  | 2 mm. | 120 cc. | 10%  |             | 470   | 540  | 115/210   |       | 3½           | 95  |
|    | 2   | 536   | 570  | 2 mm. | 120 cc. | 10%  |             | 485   | 560  | 126/210   |       | 3½           |     |
|    | 3   | 543   | 582  | 2 mm. | 120 cc. | 10%  |             | 490   | 570  | 130/210   |       | 4+           |     |
|    | 4   | 550   | 588  | 2 mm. | 120 cc. | 10%  |             | 500   | 575  | 137/210   |       | 4½           |     |
|    | 5   | 561   | 598  | 2 mm. | 120 cc. | 10%  |             | 510   | 595  | 139/210   |       | 4½           |     |
|    | 6   | 572   | 615  | 2 mm. | 120 cc. | 10%  |             | 525   | 610  | 144/210   |       | 4½+          |     |
|    | 7   | 584   | 629  | 2 mm. | 120 cc. | 10%  |             | 550   | 630  | 155/210   | (+2)  | 4½           |     |
|    | 8   | 600   | 650  | 2 mm. | 120 cc. | 10%  |             | 560   | 640  | 159/210   | (+6)  | 5½           |     |
| 25 | 9   | 644   | 780  | 2 mm. | 120 cc. | 10%  |             | 575   | 640  | 162/210   | (+20) | 6½           | 100 |

distillate from the last one or more vaporizers. On the other hand, the production of distillates having the extremely high flash and fire tests of distillate IV is not ordinarily required.

The following is a distillation analysis of distillate II. Cuts were made equaling ten per cent. fractions. The vapor temperature is recorded in the first column and the liquid temperature in the second column; these temperatures being those at the ends of the distillation of the respective fractions. The oil started to distil at a liquid temperature of 600° F. and at a vapor temperature of 500° F. under two millimeters mercury absolute pressure. The last ten per cent. fraction could not be distilled.

Gravity 17.7; flash 540°; fire 640°; viscosity 196/210.

Charge 1200 cc.  
Initial 500—600 at 2 mm.

It will be noted that even the blended distillate has very high flash and fire tests with excellent color; and that the first 10% fraction has a flash point not lower than 470° F. and a fire point not lower than 540° F. and that the ninth 10% fraction has a flash point not lower than 575° F. and a fire point not lower than 640° F.

It will also be noted that even the blended distillate has fire and flash points so high that the proportion of the lower boiling blended distillate may be increased and yet produce an oil having characteristics heretofore unknown in mineral lubricating oil distillates.

The characteristic features of the improved oil may be enumerated as follows: An oil having a flash point within the range 480°—575° F. and preferably over 500° F., a fire point within the range 560°—660° F. and preferably over 580° F. and being further characterized by the fact that

| 50 | Cut        | Temp. |      | Pres. | Am't.     | Chg. | Crude grav. | Flash | Fire | Viscosity | C.T. | Color N.P.A. | 125 |
|----|------------|-------|------|-------|-----------|------|-------------|-------|------|-----------|------|--------------|-----|
|    |            | Vap.  | Liq. |       |           |      |             |       |      |           |      |              |     |
| 55 | 1          | 588   | 632  | 2 mm. | 120 cc.   | 10%  |             | 480°  | 540° | 143/210   |      | 6½           |     |
|    | 2          | 596   | 642  | 2 mm. | 120 cc.   | 10%  |             | 510   | 560  | 162/210   |      | 6            |     |
|    | 3          | 600   | 648  | 2 mm. | 120 cc.   | 10%  |             | 530   | 615  | 184/210   |      | 6            |     |
|    | 4          | 610   | 655  | 2 mm. | 120 cc.   | 10%  |             | 520   | 630  | 188/210   |      | 5½           | 130 |
|    | 5          | 614   | 672  | 2 mm. | 120 cc.   | 10%  |             | 530   | 640  | 175/210   |      | 5½           |     |
|    | 6          | 616   | 676  | 2 mm. | 120 cc.   | 10%  |             | 550   | 650  | 179/210   |      | 6            |     |
|    | 7          | 622   | 672  | 1 mm. | 120 cc.   | 10%  |             | 540   | 645  | 185/210   |      | 6½           |     |
|    | 8          | 636   | 688  | 2 mm. | 120 cc.   | 10%  |             | 560   | 660  | 210/210   |      | 6½           |     |
|    | 9          | 655   | 718  | 2 mm. | 120 cc.   | 10%  |             | 585   | 680  | 231/210   |      | 6½           |     |
| 60 | B. t. m's. |       |      |       | 1,200 cc. | 100% |             | 640   | 710  | 323/210   |      |              | 135 |

It will be noted that all the distilled oils I, II, III and IV have a flash point not less than 535° F. and a fire point not less than 625° F. Distillate IV merely illustrates how much higher it is possible, in my process, to carry the flash and fire points. Distillation analyses of distillates I, II and III show that the first ten per cent. is characterized by having a flash point not lower than 480° F. and a fire point not lower than 540° F. and that the ninth 10% fraction has a flash point not lower than 580° F. and a fire point not lower than 680° F.

The flash and fire points of these oils are, it is believed, far higher than those characterizing

its Conradson carbon content does not exceed seven-tenths of one per cent. (.007), that its color is not more than 7½ N. P. A., that the oil is neutral, that is, its organic acidity as tested by the A. S. T. M. method does not exceed two-hundredths and that it has a good demulsibility test in accordance with the Herschel method, i. e., between 1550 and 1620.

The Conradson carbon content will vary with the crude. Oils of the flash and fire points herein described, produced as herein described, vary in their Conradson carbon content, from .4 to less than one percent. In the case of the particular crudes herein mentioned the Conradson

carbon content of the oils produced as herein described is between .5 and .7 percent.

It is known to produce distillates of low flash, fire and viscosity having a Conradson carbon content substantially less than one percent. It is also known to produce distillates having low flash, fire and viscosity that have low organic acidity. It is also known to produce residual (cylinder) oils having a high flash and fire (but lower, it is believed, than the minimum characterizing the oils herein described), which are neutral. It is, however, I believe, unknown to produce distillates of the high flash, fire and (or) viscosity characterizing the oils herein described, or to produce distillates of high flash, fire and (or) viscosity which are neutral, or to produce distillates or residual oils of high flash, fire and (or) viscosity which have a Conradson carbon content under one percent, and it is certainly unknown to produce distillates having all of the qualities specified.

It will be observed that certain of the characteristic features of the new oil are those possessed by high grade bright stock, which is a final, highly refined and expensive residue from paraffin base oils; but bright stock is a residual oil and lacks important and valuable characteristics of the new distillates. Thus it is impossible to reduce the carbon content of a residual oil much below one per cent. (Conradson test); nor is it possible, with a residual oil, to obtain a color comparable to that hereinbefore specified for the new distillate, except by filtration at an excessive cost. It is one of the pronounced advantages of the improved distillate that it possesses the required and desirable qualities of the best and much more expensive cylinder oil or bright stock and at the same time possesses other superiorities. Thus, a low carbon content is in itself a desideratum, while the good color is indicative of the comparative absence of undesirable products of decomposition.

For certain restricted uses the distillate from vaporizer 10 should not be blended, or should be blended with but a small proportion of oil from vaporizer 9; and an oil having a flash point of not less than 525° F. and a fire point of not less than 605° F., and with the other qualities specified, is a specific example of a very high boiling point oil that is within the broader scope of the invention.

No specific viscosity range characterizes the new distillates, inasmuch as various kinds of crudes will produce oils all having the essential qualities hereinbefore enumerated but varying greatly in viscosity. The flash and fire tests of lubricating oils of similar viscosity from different crudes will vary within rather wide limits. Thus, Vinton crude yields a fraction having a viscosity of 200 @ 210° F. with a flash point of 515° F. and fire point of 610° F. Mirando crude yields a fraction of the same viscosity having a flash point of only 470° F. and a fire point of only 510° F. The average boiling point of the fraction of Vinton crude oil at 2 mm. absolute pressure is approximately 610° F., while the average boiling point of the fraction of Mirando crude oil at the same pressure is approximately 510° F.

Now it is well understood that a distillate having high fire and flash tests with a relatively low viscosity is much more desirable and valuable than a distillate having the same fire and flash tests with a relatively high viscosity. It is a characteristic feature of the process herein described that, with a given crude oil, a distillate can be

obtained that, for a given viscosity, has much higher flash and fire points than any heretofore known; but the viscosity characteristic cannot be expressed in the claims, because it necessarily varies within a wide range dependent on the crude.

Another pronounced advantage of the process by which the new distillates are produced is that it is possible to produce low viscosity and high flash and fire test distillates from crudes that heretofore could not be commercially used to produce high boiling distillates because of the too high viscosity by which they were inevitably characterized.

It should be stated that it may be possible to produce, from certain crudes, by processes heretofore known, lubricating distillates having fire and flash tests approximating the lower limit of the ranges heretofore specified as characterizing the new distillates; but such distillates, aside from flash and fire tests, are either cuts too narrow to be commercially practicable or do not have the combination of characteristics and qualities herein specified as characterizing the new distillates.

In different claims among those appended, the minimum flash and fire points are differently stated: first, because while the lower limits of the flash and fire ranges specified distinguish from all distillates known to me, they may not of themselves distinguish from distillates unknown to me; and second, one of the main objects or advantages of the invention is the production of a distillate that will possess the desirable qualities of known residual oils such as the best bright stocks; and such distillates, to meet the exacting requirements of many uses, must possess flash and fire points much higher than those within the lower part of the broadest range specified, and claims limited to distillates that are competitive with, and at the same time superior to, such residual oils are necessary in order to define the more radically novel, as well as the most commercially valuable, embodiments of this invention.

It should be understood that if a narrow cut of the new distillate is desired, this presents no difficulties, since in the process described, as many fractions as desired may be obtained by increasing the number of vaporizers, or by separately condensing the vapors escaping from different points along the length of a vaporizer, or by fractional condensation of the vapors. The higher boiling of such narrow cuts have extraordinarily high flash and fire points, but their production is not usually commercially practicable, because their abstraction necessarily reduces the flash and fire points of a blend of the remaining fractions.

Having now fully described my invention, what I claim and desire to protect by Letters Patent is:

1. A lubricating oil which is a distillate of petroleum and which has a flash point about the range 550 to 675° F. and a higher fire point within about the range 625 to 730° F. and which is further characterized by the fact that its organic acidity as tested by the A. S. T. M. method does not exceed two-hundredths neutralization number and that its Conradson carbon content is between four-tenths percent and one percent.

2. A lubricating oil which is a distillate of petroleum and which has a flash point within about the range 575 to 675° F. and a higher fire point within about the range 650 to 730° F. and which is further characterized by the fact that its organic acidity as tested by the A. S. T. M. method does not exceed two-hundredths neutralization number and that its Conradson car-

80

85

90

95

100

105

110

115

120

125

130

135

140

145

150

bon content is between four-tenths percent and one percent.

3. A lubricating oil which is a distillate of petroleum and whose components are such that when fractionally distilled its first ten per cent. fraction has a flash point within about the range 460 to 550° F. and a fire point within about the range 530 to 650° F. and that its ninth ten per cent. fraction has a higher flash point within about the range 560 to 675° F. and a higher fire point within about the range 625 to 730 F. and which is further characterized by the fact that its organic acidity as tested by the A. S. T. M. method does not exceed two-hundredths neutralization number and that its Conradson carbon content is between four-tenths percent and one percent.

4. A lubricating oil which is a distillate of petroleum and which has a flash point within about the range 500 to 640° F. and a higher fire point within about the range 590 to 710° F. and which is further characterized by the fact that the boiling point range between the initial boiling point and the boiling point at the end of the ninth ten per cent. fraction is not less than about 60° F., that its organic acidity as tested by the A. S. T. M. method does not exceed two-hundredths neutralization number and that its Conradson carbon content is between four-tenths percent and one percent.

5. A lubricating oil which is a distillate of petroleum and which has a flash point within about the range 500 to 600° F. and a higher fire point within about the range 590 to 700° F. and which is further characterized by the fact that the boiling point range between the initial boiling point and the boiling point at the end of the ninth ten percent fraction is not less than about 100° F., that its organic acidity as tested by the A. S. T. M. method does not exceed two-hundredths neutralization number and that its Conradson carbon content is between four-tenths percent and one percent.

45 6. A lubricating oil which is a distillate of petroleum and which has a flash point within about the range 500 to 640° F. and a higher fire point within about the range 590 to 710° F. and which is further characterized by the fact that the boiling point range between the initial boiling point and the boiling point at the end of the ninth ten per cent. fraction is not less than about 50 60° F., that its Conradson carbon content is between four-tenths percent and one percent and that its organic acidity as tested by the 55 A. S. T. M. method does not exceed two-hundredths neutralization number.

60 7. A lubricating oil which is a distillate of petroleum and which has a flash point within about the range 510 to 640° F. and a higher fire point within about the range 595 to 710° F. and which is further characterized by the fact that the boiling point range between the initial boiling point and the boiling point at the end of the ninth ten percent fraction is not less than about 60° F., that its organic acidity as tested by the A. S. T. M. method does not exceed two-hundredths neutralization number and that its Conradson carbon content is between four-tenths percent and one percent.

8. A lubricating oil which is a distillate of petroleum and which has a flash point within about the range 510 to 600° F. and a higher fire point within about the range 595 to 700° F. and  
75 which is further characterized by the fact that

the boiling point range between the initial boiling point and the boiling point at the end of the ninth ten percent fraction is not less than about 100° F., that its organic acidity as tested by the A. S. T. M. method does not exceed two-hundredths neutralization number and that its Conradson carbon content is between four-tenths percent and one percent.

9. A lubricating oil which is a distillate of petroleum and which has a flash point within about the range 510 to 600° F. and a higher fire point within about the range 595 to 700° F. and which is further characterized by the fact that the boiling point range between the initial boiling point and the boiling at the end of the ninth ten per cent. fraction is not less than about 100° F., that its Conradson carbon content is between four-tenths percent and one percent and that its organic acidity as tested by the A. S. T. M. method does not exceed two-hundredths, neutralization number. 95

10. A lubricating oil which is a distillate of petroleum and which has a flash point within about the range 525 to 640° F. and a higher fire point within about the range 610 to 710° F. and which is further characterized by the fact that the boiling range between the initial boiling point and the boiling point at the end of the ninth ten per cent. fraction is not less than about 60° F., that its organic acidity as tested by the A. S. T. M. 100  
method does not exceed two-hundredths neutralization number and that its Conradson carbon content is between four-tenths percent and one percent. 105

11. A lubricating oil which is a distillate of petroleum and which has a flash point within about the range 525 to 600° F. and a higher fire point within about the range 610 to 700° F. and which is further characterized by the fact that the boiling range between the initial boiling point and the boiling point at the end of the ninth ten per cent. fraction is not less than about 100° F., that its organic acidity as tested by the A. S. T. M. method does not exceed two-hundredths neutralization number and that its Conradson carbon content is between four-tenths percent and one percent.

12. A lubricating oil which is a distillate of petroleum and which has a flash point within the range 550 to 640° F. and a higher fire point within about the range 625 to 710° F. and which is further characterized by the fact that the boiling range between the initial boiling point and the boiling point at the end of the ninth ten per cent. fraction is not less than about 60° F., that its organic acidity as tested by the A. S. T. M. method does not exceed two-hundredths neutralization number and that its Conradson carbon content is between fourth-tenths percent and one percent. 125 130 135

13. A lubricating oil which is a distillate of petroleum and which has a flash point within the range 575 to 640° F. and a higher fire point within about the range 650 to 710° F. and which is further characterized by the fact that the boiling range between the initial boiling point and the boiling point at the end of the ninth ten per cent. fraction is not less than about 60° F., that its organic acidity as tested by the A. S. T. M. method does not exceed two-hundredths neutralization number and that its Conradson carbon content is between four-tenths percent and one percent.